

(No Model.)

T. S. VERY.

INGOT FOR THE MANUFACTURE OF COMPOUND METALLIC TUBES.

No. 371,719.

Patented Oct. 18, 1887.



WITNESSES.

A. D. Grover—  
C. D. Foster

INVENTOR.

The S. Very.  
By Wright, Brown & Crossley,  
S. " atty.

# UNITED STATES PATENT OFFICE.

THEODORE S. VERY, OF BOSTON, MASSACHUSETTS.

## INGOT FOR THE MANUFACTURE OF COMPOUND METALLIC TUBES.

SPECIFICATION forming part of Letters Patent No. 371,719, dated October 18, 1887.

Application filed June 27, 1887. Serial No. 242,638. (No model.)

*To all whom it may concern:*

Be it known that I, THEODORE S. VERY, of Boston, in the county of Suffolk and State of Massachusetts, have invented certain new and useful Improvements in Ingots for the Manufacture of Compound Metallic Tubes, of which the following is a specification.

My invention relates to the manufacture of metallic tubes, and has as its object the construction in an economical and practical manner of compound hollow ingots or blanks from which such tubes may be rolled or formed, which, in addition to being stronger and less liable to breakage than welded tubes, may have a smoother finish on the inside, and in some cases and for some uses be practically non-corrosive—as, for example, in boilers of steam-engines, ordinary tubes of iron or steel in such cases having to be frequently cleaned and replaced on account of oxidation and accumulations of rust and scale. By my improved process tubes for boilers, axles, shafting, or any other article constructed as a tube of metal may be formed having a wrought-iron lining or inside 15 coating and an outside covering or coating of mitis, iron or steel, or vice versa. Compound tubes of brass and copper, or copper and iron, or iron and brass, or copper and steel, or other compounds or combinations, may be formed in accordance with my process, and in like manner 20 tubular ingots may be cast so that the two or more metals composing the same may be intimately and firmly united or welded together.

I will now proceed to describe my invention, so that others skilled in the art may understand and practice or use it, reference being made to the accompanying drawing, and to the letters of reference marked thereon, forming a part of this specification, which drawing 25 shows a vertical section of a mold and its contained castings, illustrating my invention.

In carrying out my invention I take a tube, *a*, of any desired metal, having thick or thin walls, as may be required for the purpose for 30 which the compound tube or casting is intended, and after heating it regularly in a proper furnace to a sufficient degree I stand

said tube *a* in a mold, *b*, of any form or construction suited to the purpose, and immediately pour around it the molten metal, *c*, intended for the outer coating or covering, which metal *c*, being at a higher degree of heat than the tube *a*, raises the degree of heat of the latter to a point effecting a substantial fusion and thoroughly effective welding of the two 50 metals at their meeting line.

If the inner tube *a* should be thin, so as that it would warp or yield to the pressure of the molten metal, a piece of round iron or steel may be placed in the tube before placing the 55 latter in the mold, which round piece of metal may be withdrawn after casting.

In some instances in practicing my invention I paint or surround the tube with a coating containing a sufficient quantity of flux— 60 borax or other compound containing it—and, after placing the tube while thus coated in the mold, pour the molten metal around it, as described. After the casting so formed has been finished it may be allowed to cool, and 65 be subsequently heated in order to treat it by rolling, or otherwise treated for the purpose of enlarging, lengthening, or expanding it, as 70 may be desired.

Having thus described my invention, what I 75 claim is—

1. In the art of manufacturing ingots for compound metallic tubes, the improvement 80 consisting in heating a metallic tube, then placing such heated tube in a mold, and finally pouring molten metal in the mold around the tube, whereby the molten metal will be united to the tube, as set forth.

2. In the art of manufacturing ingots for compound metallic tubes, the improvement 85 consisting in coating a metallic tube with a suitable flux, then placing such tube in a mold, and finally pouring molten metal in the mold around the tube, whereby the molten metal will be united to the tube, as set forth. 90

3. In the art of manufacturing compound metallic tubes, the improvement consisting in placing a metallic tube in a mold, then pouring molten metal in the mold around the tube,

and finally rolling or otherwise treating the article so formed to construct a tube of desired dimensions, as set forth.

4. An ingot for the manufacture of a compound metallic tube or tube composed of two or more kinds of metals, said metals being intimately connected or united at their line of meeting by fusing, as set forth.

In testimony whereof I have signed my name to this specification, in the presence of two subscribing witnesses, this 24th day of June, A. D. 1887.

THEODORE S. VERY.

Witnesses:

ARTHUR W. CROSSLEY,  
C. F. BROWN.